

April 3, 1956

A. L. BALL

**2,740,725**

## MANUFACTURE OF FLEXIBLE ABRASIVE PRODUCTS

Filed July 2, 1953

2 Sheets-Sheet 1

Fig. 1



*INVENTOR.*  
*ALBERT L. BALL*

BY *Ashland F. Harlan, Jr.*  
ATTORNEY

April 3, 1956

A. L. BALL

2,740,725

MANUFACTURE OF FLEXIBLE ABRASIVE PRODUCTS

Filed July 2, 1953

2 Sheets-Sheet 2

Fig 2



Fig 5



Fig 3



Fig 6



Fig 4



INVENTOR.  
ALBERT L. BALL

BY *Askan J. Harlan Jr.*  
ATTORNEY

2,740,725

## MANUFACTURE OF FLEXIBLE ABRASIVE PRODUCTS

Albert L. Ball, Worcester, Mass., assignor to Bay State Abrasive Products Company, Westboro, Mass., a corporation of Massachusetts

Application July 2, 1953, Serial No. 365,721

5 Claims. (Cl. 117—20)

This application relates to flexible abrasive products. It is particularly concerned with the manufacture of such products which comprise an open mesh fabric base with deposits of abrasive granules adhesively held on the exposed surfaces of the yarns of the fabric.

It is an object of the invention to provide an improved and efficient method for the production of flexible abrasive products of the character described.

Another object of the invention is to provide a method for the production of flexible abrasive products of the character described which results in more uniform and durable products.

Other objects and advantages of the present invention will be apparent from the following specification taken in conjunction with the accompanying drawing in which:

Figure 1 is a view diagrammatically illustrating apparatus by which the abrasive products of the character described may be produced according to the present invention;

Figure 2 is an enlarged, fragmentary, diagrammatic view of a portion of the apparatus shown in Figure 2;

Figure 3 is an enlarged plan view of a portion of a flexible abrasive product made in accordance with the method of the present invention, a portion of the open mesh fabric base being shown without an abrasive deposit thereon;

Figure 4 is a sectional view taken on line 4—4 of Figure 3;

Figure 5 is an enlarged plan view of a portion of another type of open mesh fabric which may be used as a base in carrying out the process of the present invention; and

Figure 6 is a sectional view taken on line 6—6 of Figure 5.

The process of the present invention provides an improved method by which the flexible abrasive articles or products described in copending application, Serial No. 365,722 filed July 2, 1953 may be more uniformly and satisfactorily produced. An example of such an abrasive product is illustrated in Figures 3 and 4 of the present application. It comprises an open mesh fabric base having a plurality of interlaced warp yarns 11 and filling yarns 13, the entire exposed surfaces of the yarns being covered with a deposit 15 of abrasive granules. In the illustration, a part of the open mesh fabric base is exposed by removal of the abrasive deposit from portions of the yarns.

The fabric base employed in forming the flexible abrasive product is preferably woven from continuous filament yarns. Preferably, also, the fabric after weaving and before application of the abrasive deposit is coated or pre-sized with a flexible material. The yarns are thereby not only coated, but are caused to adhere at their points of interlacing so that slipping or shifting of the yarns will be substantially prevented. When the yarns of the fabric base are of the multiple filament type

they are also impregnated to a greater or less extent. Such impregnation is usually desirable as the yarns are thus rendered substantially non-absorbent and, consequently, are not penetrated by the adhesive or bond used for applying the deposit of abrasive granules thereto. Since the bond employed is preferably rather hard, rigid and brittle, the flexibility of the abrasive product is improved if the bond is not allowed to penetrate into the fabric yarns.

10 According to the present improved method of producing a flexible abrasive article such as is illustrated in Figure 3, an open mesh fabric web, previously pre-sized as described above, is coated with a liquid adhesive or bonding material. Abrasive granules are then impelled or projected against both sides of the adhesive coated web while the web itself is rapidly vibrated. Following the application of the abrasive granules, the web is heated to set the adhesive and is then given a coat of a liquid sizing adhesive. Another heat treatment is thereafter provided to cure the adhesives and thereby firmly secure the abrasive granules to the exposed surfaces of the yarns of the fabric.

15 In Figure 1 there is diagrammatically shown an arrangement of apparatus suitable for carrying out the novel process of the present invention. The assembly includes apparatus for applying adhesive to the web before and after the deposit of abrasive granules is applied, web-vibrating apparatus, abrasive-applying means, and driers or heaters.

20 30 In carrying out the process of the invention with the apparatus shown, the open mesh pre-sized fabric web 17 is fed from a roll 19 through an adhesive tank or vat 21 in which the yarns of the fabric receive a coating of a suitable liquid adhesive or bond. Although other adhesives may be employed, it is preferred to use a phenolic resin adhesive such as an A-stage phenol-formaldehyde liquid resin. From the adhesive tank 21 the web 17 passes between squeeze rolls 23 which are adjusted to regulate properly the amount of bond left on the fabric

25 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9

abrasive deposit on the upper surfaces of the yarns. Those abrasive granules which are not captured pass through the relatively large mesh openings of the fabric web. In so doing, some of the granules will adhere to the sides of the adhesive coated yarns. Much of the remainder of the abrasive fed from the hopper 29 is caught as it falls through the web 17 by the rotating propeller 33 and is forcibly thrown upwardly against the bottom of the web where a sufficient number of granules are captured by the adhesive coating on the lower surfaces of the yarns to give an abrasive coating on the latter.

It has been found that the results are further improved when the web 17 is vibrated during deposition of the abrasive granules thereon. Adjacent to the abrasive application zone which comprises abrasive hoppers 29 and 39, therefore, the web passes between vertically spaced vibrating jaws 35 and 37 and is thus caused to oscillate rapidly in a vertical direction. Such vibration not only assists in causing abrasive granules which have not adhered to the adhesive coating yarns to pass through the openings in the fabric web, but also shakes off abrasive granules which are insecurely adhered to the yarns and thus permits other granules to be brought into contact with the adhesive on the yarns so that a well-adhered, uniform deposit of abrasive may be obtained. Abrasive granules that do not adhere to the yarn surfaces accumulate in the hopper 39 and may be withdrawn therefrom and reused.

After the application of the abrasive deposit to the adhesive coated open mesh fabric web 17, the adhesive or bond is hardened. Since the web carries an abrasive deposit on both sides, it is very desirable to avoid contact of web with any support before hardening of the adhesive. Consequently, the web is passed directly into a curing zone that may comprise a drying oven 41 which is preferably relatively short in length and is there heated without support to a temperature sufficiently high as to quickly harden or cure the adhesive to such a state that the web may be passed over the supporting roller 43 at the exit end of the oven without damage to the abrasive deposit.

Sizing adhesive is then applied to the abrasive coated web 17 by passing the web through a tank or vat 45 in which the liquid adhesive is contained. When emerging from the tank 45 the web passes between squeeze rolls 47, that preferably are covered with absorbent material to remove excess adhesive, and is then again heated by passage through a second oven 49 in which both adhesive coats are cured. At the outlet end of the oven 49 the finished abrasive product passes over the roll 51 and may be wound on a reel 53.

As previously stated, the open mesh fabric base used for forming the flexible abrasive products with which the present invention is concerned, is preferably woven from continuous filament yarns. Among the yarns of this type which may be used are organic ones such as those of rayon, nylon and other organic synthetic fibrous materials as well as inorganic ones such as glass fiber yarns. Spun yarns derived from staple fibers such as cotton, linen and wool and some types of rayon, nylon and other synthetic fibers including glass fibers are not in general suitable for making a fabric base for the abrasive products of the present invention. This is a result of the tendency of the fiber ends in spun yarns to project into and partially obstruct the mesh openings, thus making the abrasive deposit uneven and irregular.

Although a leno or gauze weave may be used in forming the open mesh fabric used as a base for the abrasive products with which the present invention is concerned, it is preferred to employ a simple plain or twill weave, open mesh fabric. Such fabrics not only are less expensive to make, but may be produced with more even surfaces than fabrics having a leno or gauze weave. In consequence, their use permits the manufacture of flex-

ible abrasive products having fewer surface irregularities. Excessive surface irregularity causes undesirable deep scratches on surfaces being smoothed or polished.

- The fabric shown in Figures 3 and 4 illustrates plain weaving, each pick or filling yarn 13 passing over and under alternate ends or warp yarns 11 across the width of the cloth. Alternately, the picks pass over the odd and under the even warp yarns and under the odd and over the even warp yarns.
- 10 The twill weave differs principally from the plain weave in that in the former each filling yarn interlaces from two to four warp yarns and on each successive pick the filling yarn moves the design one step to the left or right, as the case may be, thus forming a diagonal pattern in the fabric. A twill fabric in which each filling yarn passes over two ends and then under two ends, repeating this sequence across the width of the fabric is known as a "two and two" twill. Also, since an equal number of warp and filling yarns are shown in the recurring pattern, 15 it is classified as an "even" twill. Even twills such as "two and two," "three and three," and "four and four" twills are alike on both sides and are uniform except for the diagonal mentioned above that is characteristic of twill weaves. The diagonal pattern of open mesh fabrics 20 with a twill weave makes them advantageous as base fabrics for abrasive articles of certain types.

Open mesh fabrics woven with either the plain weave or with an even twill weave are preferred as bases for the flexible abrasive products with which this invention 25 is concerned. Uneven twills and fabrics having satin or sateen weaves are often undesirable since the opposite sides are different. Moreover, fabrics woven with satin or sateen weaves are unsatisfactory because of the long exposed yarns or floats which are their principal characteristic and which make an open mesh fabric of such a weave extremely flimsy. Pile fabrics or fabrics with fancy weaves are also unsatisfactory since the desired characteristics of the present abrasive products cannot 30 be obtained with the use of such fabrics. However, fabrics with doubled warp yarns may be employed in some cases with advantage. The twill fabric illustrated in Figures 5 and 6 shows how two small, closely adjacent warp yarns or ends 61 may be substituted for a single warp yarn. The two ends together are approximately 35 equal in size to the filling yarn 63 used and each pair of warp yarns is picked as a single end. A flatter fabric of more uniform thickness may be obtained in this way. Since the doubled warp yarns 61 are treated as a single 40 yarn the twill fabric illustrated in Figures 5 and 6 is classified as a "two and two" twill. Doubled warp yarns 45 may also be used with the plain weave or with other twill weaves.

The cloth or thread count of the base fabric employed 50 in carrying out the process of the present invention may vary over a considerable range. For many purposes, a fabric having a count of about 24 x 24, i. e. one with 24 meshes per inch in each direction, is suitable. In weaving such a fabric, filling yarns equivalent in size to about 300 denier rayon yarn may be used quite satisfactorily with single warp yarns of approximately the same size or with doubled warp yarns, each of which is approximately half the size of the filling yarn. Where a flexible abrasive product of the type described herein 55 is to be made with larger mesh, or for particularly heavy duty, coarser or heavier yarns may be used. For example, in forming a 6 x 6 base fabric, yarns ranging in denier from about 1000 to 12,000 might be employed. Of course, where the product is to be used for very fine polishing, the cloth count may be somewhat greater than 60 24 x 24 and finer yarns will be preferred for forming such an open mesh fabric base. In order to permit substantial flattening at their points of interlacing the yarns in the warp and filling of the open mesh fabric base should 65 be only moderately twisted. Because, however, of the 70 75

greater tension to which the warp yarns are subjected during weaving they may be given a greater twist than the filling yarns.

The pre-sizing or coating of the open mesh fabric base referred to above may be carried out in any desired manner. Care should be taken, however, that no substantial uneven shrinkage of the fabric takes place during pre-sizing as the mesh openings of the fabric will thereby be rendered irregular in size. Various flexible materials may be used for the pre-sizing or coating of the open mesh fabric. It is preferred, however, to use a material which is substantially insoluble in water and the non-aqueous coolants that are commonly used in abrading and polishing operations. The pre-sizing material should also be substantially insoluble in the adhesive or bond used to hold the abrasive deposit on the yarns of the fabric but must be of such character that the adhesive or bond will adhere to the material remaining on the yarns as a surface coating.

Neoprene latex has been found to be suitable as a pre-sizing or coating material. It may be applied to the fabric by rolling, spraying or dipping and then dried in suitable manner to make the fabric ready for use in carrying out the present process. Other synthetic latices such as those manufactured and sold by the B. F. Goodrich Chemical Co. under the names "Geon" and "Hycar", which are aqueous dispersions of polyvinyl resins and of butadiene-acrylonitrile copolymers, respectively may be used instead of neoprene latex and solutions or emulsions of flexible plastic materials such, for example, as polyvinyl-butyl resins, polyvinyl acetate, ethyl cellulose and the like may be also employed. As previously mentioned multiple filament yarns will be impregnated by the pre-sizing material and the surface coating of the yarns will cement or tack the yarns together at their intersections, thus preventing the shifting of the yarns which is usually a serious problem in the handling of open mesh fabrics. Of course, suitable means must be provided for unblinding the mesh openings of the fabric after coating with the pre-sizing material to prevent the drying of films across the mesh openings. Obviously such films would interfere with the coating of all the exposed surfaces of the yarns with abrasive.

As mentioned above, the adhesive or bond employed in securing the abrasive deposit to the pre-sized yarns of the open mesh fabric base is preferably rather hard, rigid and brittle. Phenol-formaldehyde condensation product liquid resins have been found particularly suitable for use as such bonds. In addition to having the desirable properties mentioned, such resins after curing are also substantially insoluble and thus the abrasive products formed therewith may be satisfactorily used with coolants in wet abrading and polishing operations. Although liquid phenolic resins are preferred, other adhesive materials may be used. Among such usable materials are oil modified phenolic resin varnishes, oleo resin varnishes, and urea-formaldehyde condensation product resins. The choice of a bonding adhesive will, of course, primarily depend upon the properties desired in the abrasive product being manufactured and the other materials used.

The adhesive employed is preferably applied to the web at room temperature and a liquid adhesive having suitable viscosity for proper application within the normal range of such temperatures is therefore chosen. When employing the apparatus shown in Figure 1 the web 17 in passing from the adhesive vat or tank 21 is led between squeeze rolls 23. These rolls are adjusted to leave on the yarns of the web sufficient adhesive to permit the adherence of a thick, dense coat of abrasive granules over all the exposed surfaces of the yarns. In any particular case the amount of adhesive used will vary, of course, with the size of the yarns employed, the cloth count of the open mesh fabric base, and the size of the abrasive granules to be applied.

Although the mesh openings of the open mesh fabric

web 17 may be cleared or unblinded after application of the bond in any one of a number of ways, excellent results have been obtained by the use of a high velocity jet of gas as described above. The velocity required in 5 the jet will vary with the viscosity of the bonding adhesive employed and the size of the mesh openings. With thick or viscous adhesives a higher gas velocity will be required than is needed when thin or less viscous adhesives are used. Similarly, the unblinding of the mesh 10 openings in a fabric in which the cloth count is relatively high will usually require a higher gas velocity than is required for a fabric in which the cloth count is relatively low since the adhesive or bond films extending across the mesh openings of the fabric with the smaller openings are 15 likely to be stronger. Adjustment of the velocity of the jet or gas may be made by varying the inlet pressure to the casing 26 or by varying the width of the slot 24 by the slide 25. The velocity of the gas emitted from the slot 24 should, in any case, be regulated to that it will not 20 be greater than required to break the films of adhesive in the meshes. Higher velocities than this may displace the film of adhesive from the yarns or damage it and thus cause irregularity in the deposit of abrasive granules.

The vibration of the open mesh fabric web during application of the abrasive granules to the adhesive coated 25 yarn that has been found desirable in producing improved results may be carried out in any convenient manner. Satisfactory vibration has been secured by passing the web through a slot between closely spaced, vertically arranged jaws which extend transversely of the web. The 30 jaws are driven by any suitable means (not shown) to cause the web to oscillate rapidly in a vertical direction. The frequency of oscillation may vary and preferably is somewhat greater when fine abrasive granules are being 35 used than when coarser granules are employed. A frequency of vibration or oscillation between about 900 and 1200 cycles per minute has been found satisfactory. The amplitude of the oscillation may also vary but a small movement, of the order of  $\frac{1}{2}$  inch, has been found 40 to be generally sufficient. It is important that the jaws of the vibrating apparatus be very narrow. If jaws wider than about  $\frac{1}{4}$  inch are used the adhesive on the web may be picked up or disturbed to such an extent that the proper or desired abrasive deposit cannot be obtained. 45 Preferably, the jaws are approximately  $\frac{1}{32}$  inch in width. The distance between the jaws may vary. It should be great enough to permit free passage of the web but must obviously be relatively small if the web is to be properly vibrated.

The abrasive material used may be alumina, silicon carbide or any other desired kind of manufactured or natural abrasive or mixtures thereof. The amount of abrasive deposited as a coating on the yarns of the open mesh base fabric will vary with the amount of adhesive used, the yarn size, and the size of the abrasive granules. 55 Using a base fabric with a cloth count of 24 x 24 woven from 300 denier rayon yarns, the weight of abrasive in the deposit, for grit sizes from 600 to 280 may vary between about 7.5 lbs. to 17 lbs. per ream (9 in. x 11 in., 500 sheets). Using a base fabric with a cloth count of 60 16 x 16 woven from 900 denier yarns, the weight of a 180 grit abrasive deposit may be as great as 36 lbs. per ream.

The coating of abrasive granules is such as to cover 65 the entire exposed surfaces of the yarns of the open mesh base fabric and will, of course, vary in thickness according to the amount of abrasive in the coating. For many purposes an abrasive coating of considerable thickness is desirable. Thus, as shown with the abrasive coating 70 15 in Figure 3, the thickness may be such as to reduce the areas of the fabric mesh openings to about one-half of their original areas, or even less. The reduction in area of the mesh openings is related not only to the thickness of the abrasive coatings on the yarns but also to the cloth count and the yarn size of the fabric base, and the

size and nature of the abrasive granules used. Consequently, it will be subject to considerable variation. In some cases the abrasive coating may comprise only a substantially single layer of individual abrasive particles. For many purposes, however, the thickness of the coating is preferably such as to cause a reduction in size of the mesh openings of from about 15 to about 40 per cent. Since an open mesh structure is desired in the final abrasive product, it is important that the deposit of abrasive granules should not be so thick or so irregular as to substantially block the mesh openings.

In obtaining abrasive deposits of considerable thickness, it is preferred to use as abrasive granules irregular cemented aggregates or clusters of fine abrasive particles. The use of such clusters or aggregates not only makes it easier to obtain thick deposits of abrasive on the yarns of the base fabrics, but it also makes it possible to obtain an abrasive deposit with which fine finishes may be secured along with rapid removal of stock.

Abrasive particles may be formed into irregular bonded aggregates or clusters by any convenient method, such, for example, as that disclosed in Jackson Patent No. 2,194,472, and with any suitable bond. In the copending application referred to above there is a discussion of the factors involved in determining the suitability of a bond for the formation of abrasive aggregates or clusters to be used in flexible abrasive products of the type with which the present invention is concerned. Although the abrasive granules used in carrying out the present invention must obviously be smaller in size than the mesh openings of the base fabric on which they are to be secured, their size, whether individual particles or bonded aggregates, may vary within wide limits. The size of the abrasive particles in such aggregates may also vary and mixtures of aggregates of different sizes may be employed as well as mixtures of aggregates with individual abrasive particles.

The rate at which the abrasive particles are fed from the hopper 29 (see Figure 2) onto the adhesive coated web 17 is not particularly critical but may be controlled by the gate 30. It is desired, however, to have an excess of abrasive falling upon the web so that ample abrasive will be available for projection against the lower surface of the web by the propeller 33. The latter may be driven by any suitable means (not shown) and is equipped with vanes 34 extending outwardly therefrom which catch the particles of abrasive falling through the mesh openings of the web and forcibly project them upwardly into contact with the lower surfaces of the adhesive coated yarns forming the web. The rate of rotation of the propeller may vary with the grit size of the abrasive particles employed, such rate being preferably somewhat less with fine abrasive particles than with larger abrasive particles. The propeller will ordinarily be caused to rotate at a speed of between about 600 and 800 R. P. M.

The heating of the abrasive coated web to cure or set the adhesive is, as pointed out above, preferably carried out in an oven. The oven may be heated in any desired manner but is preferably so constructed and operated that the web is rapidly heated so as to minimize the length of the oven 41 and, consequently, the unsupported span of the web between the squeeze rolls 23 and the roller 43. It has been found convenient when using a phenol-formaldehyde liquid resin adhesive to heat the oven with hot air to a temperature of about 280° F. and to supplement the hot air heating with radiant heat supplied from suitable devices adjacent the entrance to the oven so that the temperature of the web will be quickly raised to oven temperature. It will be understood that complete cure of the adhesive bond in the oven 41 is unnecessary, it being only required that the bond be set to such a degree that the abrasive will be dislodged from the web in passing through the sizing adhesive bath in the tank 45.

The sizing adhesive or bond employed is preferably

of the same type as that employed for securing the abrasive to the fabric yarns but of somewhat lower viscosity. However, other types of adhesives may be used. A discussion of the suitability of sizing adhesives for flexible abrasive products of the type with which the present invention is concerned is to be found in the copending application referred to above. The lower viscosity of the sizing adhesive permits it to flow more readily over the irregular surface of the abrasive deposit. The amount of sizing adhesive left on the web is determined by the setting of the squeeze rolls 47. As previously mentioned, these rolls are preferably covered with absorbent material and, therefore, remove excess adhesive, leaving on the surface of the abrasive product only a film of adhesive. Consequently, when the abrasive product is cured the abrasive particles, although they are securely anchored to the yarns and are well braced, will have sharp points exposed. The abrasive product will, therefore, be capable of very efficient performance.

The sizing adhesive coating is cured in the second oven 49 by heating in any suitable manner. After the adhesive is set to such an extent that the adhesive is no longer sticky the web may, if desired, be festooned or otherwise manipulated in the oven to permit longer heating or the use of higher or lower temperatures to complete the cure of the adhesives. The curing conditions, such as the temperature and time of heating, required to obtain the desired characteristic will, of course, vary with the adhesives employed and the intended use of the product. The choice of suitable conditions is, therefore, a matter for determination in accordance with circumstances. It will be understood that, if desired, the final curing may be carried out in apparatus other than the oven 49 and in accordance with known practice and procedures used in curing other abrasive coated articles.

By the method set forth herein flexible abrasive products of the type described in the copending application mentioned above, and filed concurrently herewith by the present applicant together with Orello S. Buckner and Philip C. Tucker, may be made more efficiently and with greater uniformity. As previously mentioned, vibration of the web assists in the passage through the mesh openings of unattached or loosely attached abrasive granules. It also assists in the wetting of the abrasive granules by the adhesive. Projection of the granules against the web is helpful in obtaining good contact between the granules and the adhesive. The process may be carried out with inexpensive apparatus and with a minimum of hand labor.

It will be understood that the invention as described is subject to modification without departing from the spirit of the invention. Thus, for example, the apparatus shown and described may be changed in many details or equivalent apparatus may be used. So, also, for example may there be changes in the open mesh fabric web employed. Thus instead of being woven of multiple filament yarns, it may be formed from yarns each of which comprises only a single filament. Furthermore, the fabric base used may be woven of yarns precoated with a flexible, heat-softenable material or of heat-softenable yarns as set forth in applicant's copending application, Serial Number 365,641, filed concurrently herewith. Accordingly, the invention is not to be considered as limited by the specific details set forth herein, but it is to be interpreted as broadly as permitted by the appended claims.

65 I claim:

1. The process of manufacturing a flexible, open mesh, abrasive coated fabric having substantially unblocked mesh openings which comprises applying a hardenable adhesive to a web, said web being formed of a woven, open mesh fabric and said adhesive being applied evenly to said web in such a quantity as to provide an adhesive coating over the entire exposed surfaces of the yarns thereof; passing said web substantially horizontally through an abrasive application zone; providing, within said zone, a

substantially uniform deposit of abrasive granules on the adhesive coated surfaces of said yarns by projecting abrasive granules smaller than the mesh openings of said web against both sides of said web, an excess of abrasive granules being applied to the upper face of said web, while said adhesive is still wet and while vibrating said web in a direction normal to the plane of said web solely at a point preceding said zone, vibration of said web serving to assist passage therethrough of abrasive granules that are unattached to said adhesive coated yarns and to displace from said web abrasive granules that are insecurely adhered to said yarns; and thereafter passing said web through a curing zone in which said adhesive is hardened, said web being unsupported from a point in advance of the point at which vibration is applied thereto to a point following said curing zone and being maintained out of contact with any portion of the apparatus used from a point preceding said abrasive application zone to a point following said curing zone.

2. A process according to claim 1 in which said fabric is woven from continuous filament yarns.

3. A process according to claim 1 in which at least a portion of said abrasive granules are aggregates which comprise a plurality of bonded abrasive particles.

4. A process according to claim 1 in which adhesive is again applied to said web after passage through said curing zone and said adhesive is subsequently cured.

5. The process of manufacturing a flexible, open mesh, abrasive coated fabric having substantially unblocked mesh openings which comprises applying a heat hardenable adhesive to a web, said web being formed of an open mesh fabric woven from continuous filament yarns and said adhesive being applied evenly to said web in such quantity as to provide an adhesive coating over the entire exposed surfaces of the yarns thereof; passing said web substantially horizontally through an abrasive application zone and therein forming on the adhesive coated surfaces of said yarns a substantially uniform deposit of abrasive granules, said deposit being produced while said adhesive is still sticky and while vibrating said web in a direction normal to the plane thereof solely at a point

preceding said zone, by projecting against the upper face of said web an excess of abrasive granules of smaller size than the mesh openings of said fabric and projecting against the lower face of said web at least a portion of the abrasive granules passing through the mesh openings of said fabric web, vibration of said web serving to assist passage therethrough of abrasive granules that are unattached to said adhesive coated yarns and to displace from said web abrasive granules that are insecurely adhered to said yarns; thereafter passing said web through a heated curing zone in which said adhesive is hardened, the uniformity of the abrasive deposit on said web being maintained by suspending said web unsupported from a point in advance of the point at which vibration is applied thereto to a point following said curing zone and maintaining said web out of contact with any portion of the apparatus used from a point preceding said abrasive application zone to a point following said curing zone; and subsequently applying a second coating of adhesive to said abrasive coated yarns of said web and curing said adhesive.

#### References Cited in the file of this patent

#### UNITED STATES PATENTS

|           |                  |       |               |
|-----------|------------------|-------|---------------|
| 1,857,340 | Wyatt            | ----- | May 10, 1932  |
| 1,883,535 | Burnett          | ----- | Oct. 18, 1932 |
| 1,965,703 | Hyde             | ----- | July 10, 1934 |
| 2,123,581 | Anderson         | ----- | July 12, 1938 |
| 2,138,882 | Robie            | ----- | Dec. 6, 1938  |
| 2,196,655 | Borghetto        | ----- | Apr. 9, 1940  |
| 2,355,635 | Dubilier         | ----- | Aug. 15, 1944 |
| 2,371,605 | Carlton et al.   | ----- | Mar. 20, 1945 |
| 2,375,813 | Oglesby          | ----- | May 15, 1945  |
| 2,388,999 | Riggenbach       | ----- | Nov. 13, 1945 |
| 2,425,236 | Ferrante         | ----- | Aug. 5, 1947  |
| 2,447,374 | Smyser           | ----- | Aug. 17, 1948 |
| 2,615,477 | Crawley          | ----- | Oct. 28, 1952 |
| 2,655,895 | Abeles           | ----- | Oct. 20, 1953 |
| 2,696,445 | Schwartz et al.  | ----- | Dec. 7, 1954  |
| 2,696,847 | Cotterill et al. | ----- | Dec. 14, 1954 |